

0

April 20, 1926.

1,581,308

S. B. CHRISTY ET AL

ARTIFICIAL SHINGLE

Filed April 27, 1923



Fig. 1.

6 parts rock asphalt  
 2 .. portland cement

Fig. 2.



Fig. 3.



Fig. 4.



## WITNESSES

*Lawrence O. Harken*

INVENTOR  
 O. M. Long,  
 F. R. Drents,  
 S. B. Christy  
 BY *Marion Leo.*

## ATTORNEYS

106-9b w.  
Asphalt Rock

Patented Apr. 20, 1926.

1,581,308

any other material to which rock asphalt may be added to form an artificial shingle. The artificial shingle may be applied to a roof in the same manner as any other shingle.

## UNITED STATES PATENT OFFICE.

SIMEON BUSH CHRISTY, OF MURFREESBORO, TENNESSEE, OTTO M. LONG, OF BOWLING GREEN, AND FRED RICHARDSON BRENTS, OF LOUISVILLE, KENTUCKY.

### ARTIFICIAL SHINGLE.

Application filed April 27, 1923. Serial No. 635,076.

108-8

To all whom it may concern:

Be it known that we, SIMEON BUSH CHRISTY, a citizen of the United States, and a resident of Murfreesboro, in the county of Rutherford and State of Tennessee, OTTO MILTON LONG, a citizen of the United States, and a resident of Bowling Green, in the county of Warren and State of Kentucky, and FRED RICHARDSON BRENTS, a citizen of the United States, and a resident of Louisville, in the county of Jefferson and State of Kentucky, have invented certain new and useful Improvements in Artificial Shingles, of which the following is a specification.

This invention relates to artificial shingles and has for its object a product and process for forming the product from rock asphalt.

Shingles have been made of a mixture of liquid or viscous asphalt which has been heated sufficiently to get the proper miscibility of the asphalt and then pressed into shape by any well known means. Reinforcing elements have been added to the asphalt either by running the reinforcing means through liquid asphalt or by pressing the same into the melted asphalt when in the process of forming the shingles.

It is an object of our invention to form a shingle of asphalt without the use of heat and in which the shingle is formed of finely ground rock asphalt which is pressed to the desired thickness whereby the shingles may be readily handled without breaking and when applied to a roof will be more durable than the artificial shingles now in use.

Other objects and advantages will become apparent during the course of the following description.

The invention is illustrated by way of example in the accompanying drawings, in which,

Figure 1 is a view in perspective of the shingles applied in overlapping relation to a roof.

Figure 2 is a transverse section of a shingle showing the manner of reinforcing the same.

Figures 3 and 4 show transverse sections disclosing other modifications of the reinforcement.

In order to form the basic shingle, we grind up rock asphalt to form a meal and this meal is placed in molds and compressed to form a shingle of sufficient thickness and flexibility that will be very durable. The rock asphalt meal may be rolled instead of being compressed to the proper size into flat sheets and the same may be cut in desired lengths and widths and where desired the sheets may be employed alone for roofing purposes.

The natural rock asphalt is employed as obtained from its natural formation in this and other countries and is therefore not a composition as is commonly employed in the construction of artificial shingles. Artificial coloring matter and cements of different kinds may be employed as desired together with any form of reinforcing element to add to the strength of the roof shingle, tiling or insulation.

Referring more particularly to the drawings, 1 indicates an asphalt shingle which is laid in overlapping relation and is formed of ground rock asphalt compressed to the desired thickness. Any form of reinforcing may be employed such as a sheet of asbestos 2 shown in Figure 2, the sheets being spaced from each other and with an intermediate reinforcing wire fabric 3.

The reinforcing sheets may be dispensed with and a wire fabric 4, disclosed in Figure 3, of the shingle 1<sup>a</sup> may be employed.

In Figure 4 a still further modified form of shingle 1<sup>c</sup> is disclosed with a single sheet of the reinforcing element 2. The wire fabrics of Figures 2 and 3 as shown more clearly in Figure 1, are embedded in the compressed asphalt of the shingle.

In Figure 1 part of the shingle 1<sup>c</sup> is cut away to disclose the sheet of asbestos 2 embedded in the compressed ground rock asphalt.

The rock asphalt employed in the construction of the shingle is a pure silicious sand thoroughly impregnated with natural asphalt. Asbestos may be employed in the finely divided state as forming part of the completed shingle or the shingle may be formed by using a 6 parts natural rock asphalt and 2 parts Portland cement.

It has been found by actual experiment that the compressed rock asphalt forms a more durable and lasting shingle and is more water-proof than the usual mixture now in common use.

While we refer specifically to shingles and disclose the same in overlapping relation in Figure 1, it must be borne in mind that the invention is not limited merely to such a construction since the rock asphalt may be

compressed in the form of tiling and employed as such.

What we claim is:

A shingle comprising a sheet of 6 parts natural rock asphalt and 2 parts Portland 15 cement.

SIMEON BUSH CHRISTY.

OTTO M. LONG.

FRED RICHARDSON BRENTS.